

Patented July 21, 1925.

1,546,367

# UNITED STATES PATENT OFFICE.

KENNETH R. BROWN, OF TAMAQUA, PENNSYLVANIA, ASSIGNOR TO ATLAS POWDER COMPANY, OF WILMINGTON, DELAWARE, A CORPORATION OF DELAWARE.

## PERCHLORATE EXPLOSIVE CONTAINING NITROGUANIDINE.

No Drawing.

Application filed March 11, 1924. Serial No. 698,573.

To all whom it may concern:

Be it known that KENNETH R. BROWN, citizen of the United States, of Tamaqua, Pennsylvania, residing at Tamaqua, Pennsylvania, in the county of Schuylkill and State of Pennsylvania, has invented certain new and useful Improvements in Perchlorate Explosives Containing Nitroguanidine, of which the following is a specification.

This invention relates to explosives containing an inorganic perchlorate or a mixture of inorganic perchlorates, and comprises explosives of this kind containing nitroguanidine.

Explosive compositions have been proposed and successfully used which contain a perchlorate or perchlorates. However, inorganic perchlorates are not in themselves very sensitive compounds and in order to make lower strength explosives in which the perchlorate content is comparatively low it is quite necessary that some ingredient be used in the composition which sensitizes the mixture and insures the proper detonation of the cartridge and the propagation of the explosion to other cartridges. Nitroaromatic compounds, such as trinitrotoluene, and liquid organic nitrates, such as nitroglycerine, either alone or in combination, may be used for this purpose. However, each of the compounds thus far proposed suffers from inherent objectionable features which restrict its application within rather narrow limits.

Trinitrotoluene, because of its considerable oxygen deficiency, cannot be used in sufficient amounts without imparting to the mixed explosive undesirable products of combustion. Moreover, a considerable percentage of trinitrotoluene is required to impart a satisfactory degree of propagation sensitiveness to explosives which contain only a small percentage of perchlorate. Trinitrotoluene is in itself an explosive, and the result is, in a good many cases, that the strength has been increased beyond the desired figure. The combination of the large percentage required and its relatively high cost makes trinitrotoluene inapplicable in a great number of instances. These same objections apply to a greater or lesser extent to other nitro-aromatic compounds.

Liquid organic nitrates, such as nitroglycerine, tetranitrodiglycerine, the nitro-

glycols, the nitrochlorhydrins, any of these mixed with nitrated sugars, and any mixtures of these with themselves, may be used in relatively small quantities to provide or increase the propagation sensitiveness. However, the percentage required is usually such that the characteristic headaches caused from handling the above mentioned compounds are not avoided. Moreover, most of the above mentioned liquid organic nitrates, when used in any considerable amounts, cause the mixed explosive to freeze at relatively high temperatures.

The use of a combination of a nitroaromatic compound and a liquid organic nitrate effects some improvement, but in general great enough percentages of either must be used that the disadvantages of one or the other, or both, which were pointed out above, persist in the mixed explosive. Especially, is this true where a low strength explosive is desired.

I have discovered that nitroguanidine increases the propagation sensitiveness of perchlorate explosives. Nitroguanidine is represented by the following graphic formula:



Calculation shows the oxygen deficiency of pure nitroguanidine to be minus 30.6 per cent. This compound is more desirable than trinitrotoluene in that it has a less oxygen deficiency. Trinitrotoluene is minus 74.0 per cent. Nitroguanidine is more desirable than nitroglycerine in that it is a solid compound and cannot freeze, and moreover produces no headache upon being handled. But what is of primary and greater importance, and which fact I have discovered and proven by numerous and exhaustive tests, is that nitroguanidine in relatively small amounts imparts to mixed perchlorate explosives a satisfactory degree of propagation sensitiveness. This applies to low strength as well as to high strength explosives.

Nitroguanidine may also be used in combination with other explosives such as trinitrotoluene, and nitroglycerine, and related explosives, to sensitize perchlorate explosives. When nitroguanidine is used, the percentage of trinitrotoluene or nitroglycerine, either or both, which is required, is of course reduced. Various combinations of nitroguan-

idine, trinitrotoluene and nitroglycerine, or explosives related to the last named two, produce a desirable range of results from the standpoint of density and velocity of detonation. However, for my purposes, I limit the use of nitroglycerine or related explosives to not more than 3.5 percent.

With respect to stability toward heat and storage, sensitiveness to impact, shock, or friction, numerous tests have shown that nitroguanidine imparts no undesirable properties to the mixed explosives.

Examples of formulae showing the use of nitroguanidine are given below.

|    |                          |    |
|----|--------------------------|----|
| 15 | 1. Ammonium perchlorate  | 35 |
|    | Manganese dioxide        | 6  |
|    | Nitroguanidine           | 25 |
|    | Sodium nitrate           | 28 |
| 20 | Ground coal              | 5  |
|    | Calcium carbonate        | 1  |
| 25 | 2. Potassium perchlorate | 25 |
|    | Ammonium perchlorate     | 24 |
|    | Manganese dioxide        | 4  |
|    | Nitroguanidine           | 20 |
|    | Sodium nitrate           | 19 |
|    | Ground coal              | 7  |
|    | Calcium carbonate        | 1  |
| 30 | 3. Ammonium perchlorate  | 25 |
|    | Manganese dioxide        | 4  |
|    | Nitroguanidine           | 8  |
|    | Trinitrotoluol           | 23 |
|    | Sodium nitrate           | 38 |
|    | Wood meal                | 1  |
| 35 | 4. Ammonium perchlorate  | 20 |
|    | Manganese dioxide        | 2  |
|    | Nitroguanidine           | 6  |
|    | Nitroglycerine           | 2  |
| 40 | Trinitrotoluol           | 20 |
|    | Ground coal              | 3  |
|    | Sodium nitrate           | 46 |
|    | Calcium carbonate        | 1  |

While I have given specific instances of the use of nitroguanidine and have shown definite percentages of ammonium and potassium perchlorates and nitroguanidine and other ingredients, it must be understood that I do not limit myself to these particular applications. Many changes may be made to the above examples without departing from the spirit of my invention.

For instance I specified trinitrotoluene and related explosives. Trinitrotoluene is

a nitroaromatic compound and I include the use of any satisfactory explosive nitroaromatic compound as coming within the scope of my invention.

I have specified nitroglycerine and related explosives. Nitroglycerine is an explosive liquid organic nitrate. I include within the scope of my invention, the use, within the limits specified, of any explosive liquid organic nitrate, which might be used in dynamite. This may be further defined as a material, liquid at 75° F., which when mixed with 25% of the inert substance kieselguhr and packed in an 1 1/4" x 8" dynamite cartridge can be completely detonated with a No. 6 cap. Among these explosive organic nitrates, as defined above, may be mentioned nitroglycerine, tetrinitrodiglycerine, the nitroglycols, the nitrochlorhydrins, any of these mixed with nitrated sugars, and any mixtures of these with themselves.

Having described my invention what I claim is:

1. An explosive, containing an inorganic perchlorate and up to three and one-half percent (0.00 to 3.50%) of an explosive liquid organic nitrate, in which nitroguanidine is used as a component of the explosive composition.

2. An explosive containing an inorganic perchlorate, a nitroaromatic compound and up to three and one-half percent of an explosive liquid organic nitrate, one or more inorganic nitrates and one or more oxygen deficient materials other than a nitroaromatic compound, together with nitroguanidine.

3. An explosive containing an inorganic perchlorate, an inorganic nitrate, an explosive liquid organic nitrate and nitroguanidine.

4. An explosive containing a mixture of an inorganic perchlorate, an inorganic nitrate, an explosive liquid organic nitrate, an oxygen deficient material other than a nitroaromatic compound and nitroguanidine.

In testimony whereof he affixes his signature in the presences of two witnesses.

KENNETH R. BROWN.

Witnesses:

ROY L. HILL,  
RUSSELL M. COOK.